

Feb. 27, 1923.

1,447,071.

C. GIESECKE,

PROCESS OF AGGLOMERATING MIXTURES OF FINE ORE AND FUEL IN SHAFT FURNACES.

FILED SEPT. 26, 1922.



Inventor

Carl Giesecke,

By *James L. Morris*  
Attorney

Patented Feb. 27, 1923.

1,447,071

# UNITED STATES PATENT OFFICE.

CARL GIESECKE, OF BAD HARZBURG, GERMANY.

## PROCESS OF AGGLOMERATING MIXTURES OF FINE ORE AND FUEL IN SHAFT FURNACES.

Application filed September 26, 1922. Serial No. 590,679.

To all whom it may concern:

Be it known that I, CARL GIESECKE, engineer, a citizen of Germany, residing at Bad Harzburg, Germany, have invented certain new and useful Improvements in Processes of Agglomerating Mixtures of Fine Ore and Fuel in Shaft Furnaces (for which I have filed application in Germany, February 18, 1920), of which the following is a specification.

My invention relates to a process of agglomerating mixtures of fine ore and fuel in shaft furnaces.

The process of agglomerating blocks of fine iron ore by means of small coke within shaft furnaces in some cases yields a product which, in addition to a high degree of rigidity, shows a very high degree of porosity, as compared to the product ordinarily resulting from the sintering process. The sintering is always accompanied by a certain glazing by reason of a partial melting of the mass. In view of these facts I have made researches to ascertain under what conditions products having said desirable properties may be obtained, my object being to carry out the process in such a way as to obtain the desirable properties at will. In blast furnaces those agglomerates have the highest value which, where the solidarity of the products is the same, are the least glazed.

I have found that very porous agglomerates are obtained where the furnace is operated according to certain principles, the essential feature being that the piece or block which is not glazed in the sintering zone is thereafter brought into contact with very hot air, from which it takes up oxygen to transform the protoxid or oxid-protoxid into oxid. By thus taking up oxygen the block is transformed in a manner similar to crystallization, which transformation is effected uniformly throughout the block and results in a cementing of the individual particles to the skeleton and a corresponding increase of the volume of the particles. However, the amount of oxygen taken up by the mass is small, so that the size of the pores is not materially reduced, while the increase in rigidity caused by the oxygen is material.

The object of this invention is to operate the furnace in such a way that the process is

regularly carried out and agglomerates are obtained which have the valuable properties hereinbefore referred to. With this object in view, my invention consists in charging the shaft furnace with blocks having a small quantity of fine carbon uniformly distributed therein, rapidly heating a comparatively low layer thereof above the combustion zone while slightly sintering the same, in order to cause reduction of the iron oxid to the oxydul, and heating by means of gaseous fuel, such as flue gas, generator gas, mixed gas, or the like, said gas being supplied to the combustion zone and assisted in burning by means of ascending air.

In a modification of the process the agglomerates are subjected to a higher reducing heat by having a larger amount of carbon admixed therein, regulating the supply of gas above the combustion zone and within the latter so as to produce a larger amount of protoxid or metal, but without sintering the agglomerate at all or without sintering the agglomerate to a higher degree, and so solidifying the mass below the combustion zone by combining hot oxygen therewith by re-oxidation, while increasing the heat up to sintering temperature by running the furnace in the manner set forth.

In the accompanying diagrammatic vertical sectional view of a shaft furnace suitable for carrying out my process, 1 represents the furnace, of which the shaft preferably flares slightly downwardly and outwardly. The furnace is charged (preferably continuously as by a conveyor 2) with blocks 3 which are formed of a mixture of fine ore and a small amount of fine coke. Near the surface of the column of blocks in the furnace, ordinarily from three to six feet below said surface, gas under pressure is supplied to the furnace through nozzles 4. The amount of gas supplied through the nozzles 4 may be controlled as by a valve 5. The products of combustion are drawn off at the top of the furnace by any suitable means, as by a suction fan 6, so that air, which may be supplied by nozzles 7 or other suitable means at the lower end of the furnace, is heated by the finished blocks as they move toward the lower end of the furnace. The air, after being heated to a high temperature, arrives in the combustion zone and in contact with the gas from the nozzles 4. The

cooling zone, which is located below the gas nozzles, is preferably much higher than the part of the furnace above the nozzles 4, a suitable height being from nine to fifteen feet.

5 The finished blocks are removed as firing continues as by means of a conveyor 8.

10 The advantages of my new process, as compared to the old method wherein the ore is heated by means of solid fuel, are best illustrated by the following example: Where the ore is heated by means of solid fuel carbon is burnt, but where it is heated by means of gas mainly carbon oxid is burnt, 15 the product of the combustion being in both cases carbon dioxid. When burning carbon to produce carbon dioxid one kilogram of oxygen is developed.

$$20 \quad 8080 \cdot \frac{12}{32} = 3030 \text{ calories.}$$

But when burning carbon oxid to produce carbon dioxid one kilogram of oxygen is developed.

$$25 \quad (8080 - 2473) \cdot \frac{12}{10} = 4210 \text{ calories.}$$

Therefore, in order to develop the same amount of heat by burning carbon dioxid, 30 only 72 per cent of the volume of air is necessary, as compared to the volume of air required for burning carbon. The reduction in the volume of air required makes it possible to preheat the air to a higher temperature when ascending within the furnace and coming into contact with the sintered blocks; and, when thus heated to higher temperature, the air causes a more intense re-oxidation below the combustion zone, so much 35 40 the more because, by reason of its diminished volume, it consumes less heat in raising its own temperature. Therefore, very hot air will cause the reoxidation with such a rise of temperature that the air reaches its maximum temperature below the combustion zone, thus causing the sintering to take place below the combustion zone. However, 45 such sintering is limited to the desirable degree, because it depends on the amount 50 of oxygen passing into the ore under treatment, and the oxygen ceases to permeate the ore as the density increases.

As a matter of fact, with carbon oxid and carbon, the difference of the temperatures 55 of the preheated air is higher so far as the result is concerned, than may be assumed from the above example, as will appear from the following calculation. It may be assumed that in one case the amount of small 60 coke used in the process amounts to 8 per cent of the final sintered product, that 1 kilogram of small coke consumes 10 cubic meters of air (having regard to the necessary excess of air), that the specific heat 65 of the sintered product is on an average 0.18,

and that, in order to raise the temperature of 1 cubic meter of air 1 degree centigrade, 31 calories are required for completely and without loss transmitting the heat from the sintered product to the air. Then the temperature T of the air entering into the combustion zone is

$$T = \frac{1250 \cdot 0.18}{0.08 \cdot 10 \cdot 0.31} = 906^{\circ} \text{ C.}$$

75 For burning carbon oxid only 72 per cent of the volume of air is required, which air is therefore heated when entering into the combustion zone to  $T_1 = 1260^{\circ} \text{ C.}$

So far it has been assumed that the heat 80 is transmitted without any loss, which is practically impossible. The heat radiated from that part of the furnace which is below the combustion zone reduces the effect of the preheating of the air, so that actually the 85 above temperatures are not attained, the temperature being in case of solid fuel about  $750^{\circ} \text{ C.}$ , if the furnace is rapidly operated. Similarly the temperature of the air in case of gaseous fuel is less than  $1260^{\circ} \text{ C.}$ , and 90 it is about from 1000 to  $1050^{\circ} \text{ C.}$  Of course the temperature of  $1260^{\circ} \text{ C.}$  can not be attained, because it can in no case be more than the sintering temperature, which is about  $1250^{\circ} \text{ C.}$  However, there is a sufficiently intense reoxidation only where the 95 temperature is as high as just stated, whereas at the lower temperature of the air, where the firing is done by coke, reoxidation does not take place at all, such reoxidation being 100 observed only where the old process is practiced in connection with some products and where there has been accidental and irregular operation of the furnace.

High preheating of the air is particularly 105 important, if it is desired, by reoxidation below the combustion zone, to raise the temperature of the sintered product for the purpose of partly solidifying the same. By oxidation of 1 kilogram of iron in the compound of  $\text{FeO}$  to produce  $\text{Fe}_2\text{O}_3$ , 571 calories are set free. If it is assumed that in 1 kilogram of ore only 0.2 kilogram of Fe have 110 before been reduced to  $\text{FeO}$  and thereafter are reoxidized to  $\text{Fe}_2\text{O}_3$ , 114.2 calories are 115 set free. This heat raises the temperature of the air and of the piece of ore the specific heat of which may be set at 0.20 at the said temperature, by

$$120 \quad \frac{114.2}{0.20 + 0.8 \cdot 0.31 \cdot 0.72} = 302^{\circ}.$$

If, before the beginning of the reaction, the temperature of the air was already as high as  $1000^{\circ} \text{ C.}$ , this slight increase is sufficient 125 to raise the ore to sintering temperature, which is not more than  $1250^{\circ} \text{ C.}$ , while the temperature can be raised to  $1302^{\circ}$ . Notwithstanding this there is no melting, because the oxidation and the generation of 130

heat cease as soon as the structure of the ore has been brought to a certain density. Therefore, the furnace can be operated in a very simple manner.

- 5 Furthermore, the method has the advantage that, even a gas of low heating capacity can be used, because it is not desired to raise the temperature in the combustion zone and above the latter sufficiently to sinter the 10 blocks. The amount of heat set free by reoxidation is considerably increased when reducing iron oxid to metal, even if such reduction is effected with only a very small part of the ore. What is most important is 15 that reoxidation in the same manner as reduction takes place within the agglomerates, where also the heat is developed. Thereby high solidity is imparted to the individual agglomerates, and they have less tendency 20 to being welded together into large size blocks, as is the case where the heat required for sintering is developed by burning solid or gaseous fuel between the agglomerates.
- 25 I am aware that it is known in the art to utilize for the purpose of sintering, the heat set free by reoxidation of the ore which had previously been reduced. My process is distinguished from the known processes first, 30 in that I obtain a product of high porosity, instead of slag, and large blocks instead of small ones, second, in that I heat by means of completely burnt gas, and third, in that

I reduce by a small amount of carbon finely divided in the ore.

35

I claim:

1. The herein described process of agglomerating fine ore, which consists in mixing the ore with finely divided carbon, heating the same in a shaft furnace by means of 40 reducing gas admitted at a point near the surface of the material and below the same at a temperature insufficient to materially sinter the material and reoxidizing the ore after it has passed the combustion zone by 45 means of hot air rising in opposition to the ore.

2. The herein described process of agglomerating fine ore, which consists in mixing the ore with finely divided carbon, heating the same in a shaft furnace by means of 50 reducing gas admitted at a point near the surface of the material and below the same at a temperature substantially not higher than is necessary for reducing the ore to protoxid or metal and insufficient to materially sinter the material, and thereafter reoxidizing 55 and sintering the ore after it has passed the combustion zone by means of hot air rising in opposition to the ore.

In testimony whereof I have affixed my signature in presence of two witnesses.

CARL GIESECKE.

Witnesses:

WILHELM LEHRKE,  
WILLI FAHN.